

## 1

2,698,240

## PHOTOGRAPHIC FILMS AND THEIR PREPARATION

Francis Peter Alles, Westfield, and William Russell Saner, Plainfield, N. J., assignors to E. I. du Pont de Nemours & Company, Wilmington, Del., a corporation of Delaware

No Drawing. Application May 27, 1952,  
Serial No. 290,332

### 11 Claims. (Cl. 95—9)

This invention relates to photographic film elements. More particularly it relates to transparent photographic film elements which have a polyvinyl acetal color former-silver halide dispersion anchored to the support by means of a substratum composed of a copolymer of vinylidene chloride, an acrylic ester and itaconic acid. Still more particularly it relates to such elements wherein the film base is composed of an oriented highly polymeric linear ester of a dicarboxylic acid and a dihydric alcohol. The invention also relates to a method of preparing such elements.

An object of this invention is to provide photographic film elements wherein a polyvinyl acetal color former-silver halide dispersion is firmly anchored to a film base. Another object is to provide such elements which have improved dimensional stability. A further object is to provide such elements wherein the film base is composed of an oriented highly polymeric ester of a dicarboxylic acid and a dihydric alcohol. Still other objects will be apparent from the following description of the invention.

The use of polyvinyl acetal color formers, which are hydrophilic to water-soluble in character, as the binding agent for silver halide grains has been disclosed in a number of patents in the past six years. It has been difficult, however, to obtain adequate anchorage between thin layers composed of such dispersions and the usual types of hydrophobic film base. This is particularly true of film base composed of highly polymeric esters of dicarboxylic acids and dihydric alcohols and especially films composed of polyethylene terephthalates. These polyvinyl acetal dispersions do not have good adherence to the conventional gelatin sublayers which have been used for many years in anchoring colloid silver halide emulsion layers to hydrophobic films.

It has been found that if a hydrophobic film base is coated with a thin layer of a copolymer of vinylidene chloride, an acrylic ester and itaconic acid that this layer has excellent adherence to the film base and can be made to adhere tenaciously to a layer of polyvinyl acetal color former-silver halide dispersion in two ways, (1) by heating the coated film element to a temperature of at least 70° C. after the polyvinyl acetal silver halide dispersion layer has been applied, or (2) by first applying to the layer of copolymer a thin layer of a hydroxyl polymer which contains a plurality of recurring intralinear



groups as polymer-forming units, said polymers being water-soluble to hydrophilic in character. The adherence of the latter intermediate substratum can also be improved by heating the coated film base to a temperature of at least 70° C. before applying the silver halide dispersion. This heating step, however, can be applied after the polyvinyl acetal color-former-silver halide dispersion has been coated onto the layer of hydroxyl polymer.

Synthetic hydroxyl polymers of the water-soluble and hydrophilic type include polyvinyl alcohol and its partially substituted water-soluble lower fatty acid esters, lower alkyl esters, and lower acetals. Polyvinyl alcohol is a tough, white, amorphous material. It is soluble in water. The more highly polymerized varieties are soluble in hot water and the medium or lower polymers are soluble in cold water. They are usually prepared by hydrolysis of polyvinyl esters, such as polyvinyl acetate, polyvinyl chloracetate, polyvinyl isobutyrate, etc. The

## 2

partly hydrolyzed esters which contain a large number of recurring vinyl alcohol units



5 or free hydroxyl groups are water-soluble or hydrophilic in character and can be made by esterifying the completely or partially hydrolyzed polyvinyl acetate, etc. The polyvinyl acetals, e. g., polyvinyl acetaldehyde acetal and polyvinyl isobutyral, can be made by incomplete acetalization of polyvinyl alcohol or partially hydrolyzed polyvinyl acetate, etc.

In addition to the synthetic hydroxyl polymers just described, there may be mentioned partially and completely hydrolyzed polyvinyl ester, e. g., polyvinyl acetate,

15 copolymers with various mono-ethylenically unsaturated compounds having a terminal  $\text{CH}_2=\text{C}$  group, such as vinyl chloride, acrylic acid esters, e. g., methyl acrylate; methacrylic acid esters, e. g., methyl methacrylate; and mono-olefins, e. g., ethylene. The completely hydrolyzed ethylene/vinyl acetate interpolymers which are described in McQueen 2,397,866 and Roland 2,386,347 form an important class of synthetic hydroxyl polymers useful as binding agents for the silver halide emulsions made in accordance with this invention.

25 The solutions used to coat the substratum of the synthetic hydroxyl polymer, free from color former nuclei, may contain a coagulating agent, e. g., boric acid or a boric acid ester of a polyhydric alcohol, e. g., an ester prepared by reacting an alcohol such as ethylene glycol,

30 diethylene glycol, triethylene glycol, erythritol, sorbitol, mannitol, etc., with boric acid or a mixture of boric acid and borax, by heating the admixture to 100° C. to 160° C. A copious evolution of water occurs. The resulting products are viscous syrups or resins of a colloidal nature and have a high molecular weight and complex structure. They are readily soluble in water but are substantially insoluble in hydrocarbons but probably hydrolyze to the boric acid and glycol in water. Their preparation is described in United States Patents 1,953,741, 2,223,349, 2,223,948, 2,223,949, and 2,224,011. These compounds have been referred to as borborates.

35 In carrying out the invention a hydrophobic film which may be composed of a cellulose carboxylic acid ester, e. g., cellulose acetate, cellulose acetate propionate, cellulose acetate butyrate, cellulose nitrate, cellulose propionate; a superpolymer, e. g., a superpolyamide (nylon), an orientable highly polymeric linear ester of a dicarboxylic acid and a dihydric alcohol, e. g., polyethylene terephthalate, polyvinyl chloride, etc., is coated with a copolymer of vinylidene chloride, an acrylic ester and itaconic acid either from an organic solvent solution or from an aqueous dispersion. When an organic solvent solution is used the solvent should have only a mild solvent action on the base so that it will not appreciably dis-

40 solve the film base but have a superficial effect and merely soften or "bite" into the surface of the base. The substrata, composed of a vinyl alcohol polymer and/or the polyvinyl acetal color former-silver halide dispersion coatings are formed by coating them onto the layer of vinyl-

45 idene chloride copolymer.

45 In carrying out the invention a hydrophobic film which may be composed of a cellulose carboxylic acid ester, e. g., cellulose acetate, cellulose acetate propionate, cellulose acetate butyrate, cellulose nitrate, cellulose propionate; a superpolymer, e. g., a superpolyamide (nylon), an orientable highly polymeric linear ester of a dicarboxylic acid and a dihydric alcohol, e. g., polyethylene terephthalate, polyvinyl chloride, etc., is coated with a copolymer of vinylidene chloride, an acrylic ester and itaconic acid either from an organic solvent solution or from an aqueous dispersion. When an organic solvent solution is used the solvent should have only a mild solvent action on the base so that it will not appreciably dis-

50 solve the film base but have a superficial effect and merely soften or "bite" into the surface of the base. The substrata, composed of a vinyl alcohol polymer and/or the polyvinyl acetal color former-silver halide dispersion coatings are formed by coating them onto the layer of vinyl-

55 idene chloride copolymer.

55 In order that the three component copolymers described above will adhere to the base tenaciously and have the requisite degree of flexibility, it is essential that the initial relative proportions of monomers in the reaction mixture be within the following ranges:

| Monomer                              | Range, Percent | Preferred Range, Percent |
|--------------------------------------|----------------|--------------------------|
| Vinylidene chloride.....             | 35.0 to 96     | 75 to 95                 |
| Ethylenically unsaturated ester..... | 3.5 to 64.5    | 4 to 20                  |
| Itaconic acid.....                   | 0.5 to 25      | 1 to 5                   |

70 The useful ethylenically unsaturated esters which may be used in the copolymers are the alkyl esters of acrylic and methacrylic acids having from 1 to 18 carbon atoms in the alkyl group (e. g., methyl methacrylate, ethyl methacrylate, butyl methacrylate, octyl methacrylate, n-dodecyl methacrylate, n-octadecyl methacrylate, methyl acrylate,

## 3

ethyl acrylate and propyl acrylate; vinyl chloride, acrylonitrile and methacrylonitrile.

The monomers may be copolymerized by various methods. For example, the copolymerization may be conducted in aqueous dispersion containing a catalyst and activator, e. g., ammonium persulfate and meta sodium bisulfite, and an emulsifying and/or dispersing agent. Alternatively, the copolymers may be prepared by polymerization of the monomeric components in bulk without added diluent, or the monomers may be reacted in appropriate organic solvent reaction media. The total catalyst-activator concentration should generally be kept within a range of about 0.01% to about 2.0% by weight of the monomer charge, and preferably within a range of concentration of 0.1% to 1.0%. Improved solubility and viscosity values are obtained by conducting the polymerization in the presence of mercaptans such as ethyl mercaptan, lauryl mercaptan, tertiary dodecyl mercaptan, etc., which are effective in reducing cross-linking in the copolymer. In general, the mercaptans should be used in concentrations of 0.1% to 5.0% by weight, based on the weight of polymerizable monomers present in the charge.

The copolymers of this invention can be coated on the hydrophobic film base or support by any suitable technique, e. g., coating from a hopper, skim coating where the surface of the film passes under a roller and contacts with the surface of the liquid, coating with applicator or transfer rolls, spray coating, etc. Doctor blades, air doctor blades, etc., can be used to remove excess liquid.

The invention will be further illustrated but is not intended to be limited by the following examples.

## Example I

A sample of polyethylene terephthalate film base, having a thickness of 0.003 inch, melting point of above 200° C. and an intrinsic viscosity of 0.50 in a mixture of 2,4,6-trichlorophenol and phenol (70:100 parts by weight) was coated with an aqueous dispersion of the vinylidene chloride-methyl acrylate-itaconic acid copolymer described in Alles & Sauer U. S. patent application Ser. No. 151,274, filed March 22, 1950, now Patent No. 2,627,088. After drying at 50° C., and heating for two minutes at 100° C., the film was coated with a polyvinyl acetal color-former-silver halide dispersion, containing approximately 1.77% by weight of silver iodobromide, composed of approximately 0.9% silver iodide and 99.1% silver bromide, dispersed in the polymeric color former (4.12% by weight of the total dispersion) described in U. S. Patent 2,513,190. After drying, the silver halide dispersion was found to have good adherence to the film base. The film was exposed and processed as follows:

(1) Developed for 10 minutes at 68° F. in a solution having the following composition:

|                                       | Grams |
|---------------------------------------|-------|
| Para-aminodethylaniline hydrochloride | 2.5   |
| Sodium sulfite                        | 10.0  |
| Sodium carbonate                      | 46.8  |
| Potassium bromide                     | 2.0   |
| Water to make 1 liter                 |       |

(2) Given a 30 second rinse in water,

(3) Treated for 5 minutes at 68° F. in the following fixing bath:

|                            |       |       |
|----------------------------|-------|-------|
| Sodium thiosulfate         | grams | 240.0 |
| Sodium sulfite             | do    | 15.0  |
| Sodium tetraborate         | do    | 18.0  |
| Glacial acetic acid        | cc    | 12.0  |
| Potassium aluminum sulfate | grams | 20.0  |
| Water to make 3 liters     |       |       |

(4) Given a 5 minute rinse in water,

(5) Treated for 5 minutes at 68° F. in the following bleaching bath:

|                        |       |       |
|------------------------|-------|-------|
| Potassium ferricyanide | grams | 100.0 |
| Boric acid             | do    | 10.0  |
| Sodium tetraborate     | do    | 5.0   |
| Water to make 1 liter  |       |       |

(6) Given a 3 minute rinse in water,

(7) Given a 5 minute treatment at 68° F. in the following fixing bath:

|                       |       |       |
|-----------------------|-------|-------|
| Sodium thiosulfate    | grams | 200.0 |
| Water to make 1 liter |       |       |

(8) Given a 10 minute rinse in water.

## 4

The wet and dry anchorage, after processing, were found to be satisfactory.

## Example II

5 A second color film with a polyethylene terephthalate base of the kind described in Example I was treated as in said example except that the film was stretched biaxially after the vinylidene chloride-methyl acrylate-itaconic acid copolymer layer had been applied and before the color former emulsion was applied. The resulting film was 10 exposed and processed as described in Example I with similar results.

## Example III

A sample of a polyethylene terephthalate film base of the type used in Example I was treated with a copolymer of vinylidene chloride-methyl acrylate-itaconic acid of the type used in Example I, then stretched biaxially and coated with a solution of the following composition:

|                                                                                           | Percent |
|-------------------------------------------------------------------------------------------|---------|
| Meta - (benzoylacetamido)benzaldehyde - sodium-o-sulfobenzaldehyde-polyvinyl mixed acetal | 5       |
| Water                                                                                     | 79      |
| Methanol                                                                                  | 16      |

20 After drying at 50° C., the film was further treated with a solution of the following composition:

|                                                                                           | Percent |
|-------------------------------------------------------------------------------------------|---------|
| Meta - (benzoylacetamido)benzaldehyde - sodium-o-sulfobenzaldehyde-polyvinyl mixed acetal | 1.5     |
| Boric acid                                                                                | 1.9     |
| Diisopropanol amine                                                                       | 1.3     |
| Acetone                                                                                   | 40.0    |
| Ethyl alcohol (95%)                                                                       | 55.3    |

25 After drying at 50° C., the film was heated at 100° C. for 2 minutes and coated with a color-former dispersion of the type described in Example I. The adhesion, both wet and dry, after exposing the film and processing in the usual manner, was good. The above polyvinyl acetal is described in Example I of Martin 2,513,189.

## Example IV

A sample of a polyethylene terephthalate film base of the type used in Example I was coated with a copolymer of vinylidene chloride of the type used in Example I, dried, 45 stretched biaxially (approximately three times its original dimensions) and then coated with a solution of the following composition:

|                                                                                           | Percent |
|-------------------------------------------------------------------------------------------|---------|
| Meta - (benzoylacetamido)benzaldehyde - sodium-o-sulfobenzaldehyde-polyvinyl mixed acetal | 3       |
| Water                                                                                     | 81      |
| Methanol                                                                                  | 16      |

35 After drying at 50° C., the film was heated at 130° C. for 5 minutes and was further treated with a solution of the following composition:

|                    | Percent |
|--------------------|---------|
| Boric acid         | 1.9     |
| Diisopropanolamine | 1.3     |
| Water              | 96.8    |

40 After drying at 50° C., the film was coated with a polyvinyl acetal color-former silver halide emulsion, containing 1.77% by weight of silver iodobromide, composed of approximately 0.9% silver iodide and 99.1% silver bromide, dispersed in the polymeric color former (4.12% by weight of the total emulsion) described in Martin U. S. Patent No. 2,513,190. After drying, the emulsion was found to have good adherence to the film base. It was exposed and processed as described in Example I. Wet and dry anchorage, after processing, were good.

## Example V

A sample of a polyethylene terephthalate film base of the type used in Example I, was coated on both sides with a copolymer of vinylidene chloride of the type used in Example I, stretched biaxially, and was coated on one side with the two subbing solutions as set forth in Example III. After drying, the film was subjected to 55 a temperature of 100° C. for several minutes and was then coated with the following dispersions and solutions, in the order listed.

|                                                                                                                |
|----------------------------------------------------------------------------------------------------------------|
| (1) A polyvinyl acetal color-former-silver halide dispersion containing 1.77% by weight of silver iodobromide, |
| 55 composed of approximately 0.9% silver iodide and 99.1%                                                      |

silver bromide, dispersed in the polymeric color former (4.12% by weight of the total dispersion) described in U. S. Patent No. 2,513,190.

(2) A 1.15% solution of polyvinyl alcohol (99% hydrolyzed polyvinyl acetate, a 4% solution of which, in water, had a viscosity of 55 centipoises at 20° C.) in a mixture of water and alcohol.

(3) A polyvinyl acetal color-former-silver halide dispersion containing approximately 2.2% silver bromide dispersed in the polymeric color former (2.8% by weight of the total dispersion) described in U. S. Patent 2,489,655.

(4) The same solution given under (2).

(5) A polyvinyl acetal color-former-silver halide dispersion containing approximately 1.15% silver bromide dispersed in the polymeric color former (4.15% by weight of the total dispersion) described in U. S. Patent 2,476,988. This dispersion also contained dissolved therein, the yellow dye Tartrazine (Colour Index No. 640).

After drying, this composite light-sensitive element was found to adhere well to the film base. The film was exposed and processed as described in Example I. The wet and dry anchorage were found to be satisfactory.

While a heating temperature of at least 70° C. has been referred to above the examples include higher temperatures and indeed temperatures up to 150° C. or more can be used if they do not deleteriously affect the coated layers. This can be determined visually with respect to the particular color former. When a gelling hydroxyl polymer sublayer or non-gelling hydroxyl polymer sublayer is used the heating step may precede the application of the polyvinyl acetal color former layer.

The invention is, of course, not limited to the foregoing examples as any of the film bases referred to above may be substituted, in some cases without stretching, with similar results.

Similarly, the invention is not limited to the use of the specific polyvinyl acetal color formers given in the examples as many other hydrophilic to water-soluble acetals of this general type can be substituted with similar results. Among such additional suitable polyvinyl acetal color formers are those described in the following U. S. Patents: Jennings 2,397,864, Woodward 2,423,572, McQueen 2,464,597, Corner & Woodward 2,465,067, Martin 2,472,910, Martin 2,538,257, Martin 2,476,988, McQueen 2,477,462, Martin 2,489,655, McQueen 2,513,190, and Martin 2,518,704.

It is to be understood that in the case of color films for multicolor photography they will contain several superposed polyvinyl acetal color-former-silver halide emulsion layers which are so arranged and sensitized that they record different colors of the visible spectrum. These color formers can be selected to yield yellow, blue-green (cyan), and magenta, etc., quinoneimine, azsomethine, etc., dyes in the appropriate layers as is common in the art and described in Jennings 2,497,864 and other patents described above. Filter dyes may be present in one or more of the above color former layers or in a separate stratum, e. g., a polyvinyl alcohol or equivalent hydroxyl polymer layer as described above. In general, a yellow filter dye is used in a stratum above the two light-sensitive layers most distant from the camera side of the film.

An advantage of the invention is that it provides a simple and effective process for improving the anchorage between a polyvinyl acetal color former layer and a hydrophobic film base. Another advantage is that the process can be carried out with conventional equipment. Still other advantages will be apparent from the above.

This invention is a continuation-in-part of U. S. application Ser. No. 151,274, filed March 22, 1950.

As many widely different embodiments of this invention can be made without departing from the spirit and scope thereof, it is to be understood that the invention is not to be limited except as defined by the claims.

What is claimed is:

1. The process which comprises coating a water-permeable hydroxyl polymer layer onto a stratum composed of a tri-component copolymer made from 35 to 96% of vinylidene chloride, 3.5 to 64.5% of an ethylenically unsaturated ester and 0.5 to 25% of itaconic acid monomers, all percentages being by weight, said ester being taken from the group consisting of alkyl esters of acrylic and methacrylic acids having 1 to 18 carbon atoms in the alkyl group, acrylonitrile, methacrylonitrile and vinyl chloride: said stratum being on a hydrophobic

film base, and heating the coated layer to a temperature from 70° C. to 150° C.

2. A process as set forth in claim 1 wherein said hydroxyl polymer is a polyvinyl acetal color-former.

3. A process as set forth in claim 2 wherein said acetal has light-sensitive silver salts uniformly dispersed therethrough.

4. The process which comprises coating a water-permeable hydroxyl polymer layer onto a stratum composed of a tri-component copolymer made from 35 to 96% of vinylidene chloride, 3.5 to 64.5% of an ethylenically unsaturated ester and 0.5 to 25% of itaconic acid monomers, all percentages being by weight, said ester being taken from the group consisting of alkyl esters of acrylic and methacrylic acids having 1 to 18 carbon atoms in the alkyl group, acrylonitrile, methacrylonitrile and vinyl chloride: said stratum being on an oriented highly polymeric ester of a polymethylene glycol of 2 to 10 carbon atoms and terephthalic acid, said ester having a melting point from 200° C. to 300° C., and heating the coated base to a temperature from 70° C. to 130° C.

5. A process as set forth in claim 4 wherein said hydroxyl polymer is a polyvinyl acetal color-former.

6. A process as set forth in claim 5 wherein said acetal has light-sensitive silver halides uniformly dispersed therethrough.

7. The process which comprises coating a light-insensitive, water-permeable hydroxyl polymer layer onto a stratum composed of a tri-component copolymer made from 35 to 96% of vinylidene chloride, 3.5 to 64.5% of an ethylenically unsaturated ester and 0.5 to 25% of itaconic acid monomers, all percentages being by weight, said ester being taken from the group consisting of alkyl esters of acrylic and methacrylic acids having 1 to 18 carbon atoms in the alkyl group, acrylonitrile, methacrylonitrile and vinyl chloride: said stratum being on an oriented highly polymeric ester of a polymethylene glycol of 2 to 10 carbon atoms and terephthalic acid, said ester having a melting point from 200° C. to 300° C., heating the coated base to a temperature from 70° C. to 130° C., coating an aqueous dispersion of light-sensitive silver halides in a polyvinyl acetal color-former onto said polymer layer and drying the resulting film element.

8. The process which comprises coating a light-insensitive, water-permeable hydroxyl polymer layer onto a stratum composed of a tri-component copolymer made from 35 to 96% of vinylidene chloride, 3.5 to 64.5% of an ethylenically unsaturated ester and 0.5 to 25% of itaconic acid monomers, all percentages being by weight, said ester being taken from the group consisting of alkyl esters of acrylic and methacrylic acids having 1 to 18 carbon atoms in the alkyl group, acrylonitrile, methacrylonitrile and vinyl chloride: said stratum being on an oriented highly polymeric ester of a polymethylene glycol of 2 to 10 carbon atoms and terephthalic acid, said ester having a melting point from 200° C. to 300° C., coating an aqueous dispersion of light-sensitive silver halides in a polyvinyl acetal color-former onto said polymer layer and drying the resulting film element, heating the coated base to a temperature from 70° C. to 100° C.

9. A photographic element comprising a film base composed of an oriented highly polymeric ester of a polymethylene glycol of 2 to 10 carbon atoms and terephthalic acid, said ester having a melting point from 200° C. to 300° C., bearing in order a substratum composed of a tri-component copolymer made from 35 to 96% of vinylidene chloride, 3.5 to 64.5% of an ethylenically unsaturated ester and 0.5 to 25% of itaconic acid monomers, all percentages being by weight, said ester being taken from the group consisting of alkyl esters of acrylic and methacrylic acids having 1 to 18 carbon atoms in the alkyl group, acrylonitrile,

75 methacrylonitrile and vinyl chloride: said stratum being a layer of a water-soluble to hydrophilic hydroxyl polymer containing a plurality of intralinear —CH<sub>2</sub>—CHOH— groups as polymer units and at least one layer of light-sensitive silver halides dispersed in a polyvinyl acetal color-former.

10. A photographic element comprising a film base composed of an oriented highly polymeric ester of a polymethylene glycol of 2 to 10 carbon atoms and terephthalic acid, said ester having a melting point from 200° C. to 300° C., bearing in order a substratum com-

posed of a tri-component copolymer made from 35 to 96% of vinylidene chloride, 3.5 to 64.5% of an ethylenically unsaturated ester and 0.5 to 25% of itaconic acid monomers, all percentages being by weight, said ester being taken from the group consisting of alkyl esters of acrylic and methacrylic acids having 1 to 18 carbon atoms in the alkyl group, acrylonitrile, methacrylonitrile and vinyl chloride; said stratum being a layer of polyvinyl alcohol and at least one layer of light-sensitive silver halides dispersed in a polyvinyl acetal color-former having a plurality of intralinear —CH<sub>2</sub>—CHOH— groups as polymer units.

11. A photographic element as set forth in claim 9 wherein said alkyl ester of acrylic acid is methyl acrylate.

## References Cited in the file of this patent

## UNITED STATES PATENTS

| Number    | Name         | Date          |
|-----------|--------------|---------------|
| 2,298,039 | D'Alelio     | Oct. 6, 1942  |
| 2,491,023 | Alles et al. | Dec. 13, 1949 |
| 2,534,326 | Weaver       | Dec. 19, 1950 |
| 2,606,835 | Jennings     | Aug. 12, 1952 |
| 2,627,088 | Alles et al. | Feb. 3, 1953  |